

## UNITED STATES PATENT OFFICE

2,135,983

## METHOD OF PRODUCING BERYLLIUM ALLOYS

Menahem Merlub-Sobel, Cleveland, Ohio, assignor to The Beryllium Corporation, New York, N. Y., a corporation of Delaware

No Drawing. Application November 7, 1934, Serial No. 751,965

15 Claims. (Cl. 75—135)

This invention relates to the direct formation of beryllium alloys, particularly beryllium alloys with heavier metals, such as copper, nickel, iron, cobalt, silver, etc.

5 It has been known for many years that alloys composed of beryllium and copper possess properties of hardness and high electrical conductivity; and more recently their age-hardening properties have been discovered. This same characteristic of beryllium, that of increasing hardness and of conferring age-hardening properties upon metals, is found with others of the heavy metals—such as cobalt, nickel, iron, and ferrous alloys of varying complexity. In addition to those 10 already mentioned, alloys of beryllium with aluminum have been shown to be of great value, particularly where great lightness is desired in conjunction with relatively good strength. Similarly silver beryllium alloys have great value be- 15 cause of their resistance to tarnish.

Despite the technical advantages gained by the use of beryllium as a constituent of various alloys, commercialization of such alloys has been retarded by their high cost. This has been the inevitable 20 result of the necessity for making beryllium alloys by simple alloying of the metallic elements, the high cost of beryllium metal—a reflection of its high standing in the electromotive series—its high melting point, and lesser difficulties, such as 25 ready oxidizability, lack of fluidity, etc. Any economical utilization of beryllium in alloy form therefore necessitates the direct formation of the 30 alloys from cheap beryllium compounds instead of the present practice of alloying the elementary 35 metals.

Many attempts to accomplish this end have been made. Electro-deposition of beryllium into molten cathodes of copper, iron, etc. have been tried by numerous workers, but all with failure or 40 at best indifferent success. Codeposition of beryllium and copper has been suggested; likewise depositing alternately beryllium and copper, but no practical results have been found attainable. More recently, it has been proposed to manufacture 45 copper-beryllium alloys by beryllium formation in the presence of molten copper as a collecting agent, but it has been the applicant's experience with this procedure, even before the publication of such data, that inadequate results 50 are obtained. In all probability the same factor is here involved which acts to inhibit the formation of beryllium-copper alloys in the attempted deposition of beryllium into a molten copper cathode. In the latter case, it has been observed by 55 all workers in this field that there is so low a

tendency for alloying of the light metal into the bath of the heavy metal that comparatively little of the beryllium is captured. Even at temperatures as high as 1400° C., above the melting point of beryllium, and irrespective of whether partially alloyed copper or pure copper is used, no significant electroalloying takes place. It is therefore quite evident that, just as with a molten cathode, so a molten collecting bath will not be found satisfactory. Efforts to disperse molten copper by 10 spraying, or by colloidal action, have not succeeded, and I have therefore been led to a procedure which, though reversing normal outlooks, has nevertheless proven very successful.

If, instead of raising the temperature of the alloying metal bath, as all previous experimenters have attempted, in order to increase alloying activity, the initial temperature be reduced to below the melting point of copper, or other heavy metal employed, and if the solid copper be present in a 15 condition to present large surfaces, alloying takes place readily and smoothly. Moreover, as will be shown later, it is possible to make such a process readily continuous, thereby removing one of the 20 fatal drawbacks to economy in all beryllium operations in the past. It is to be understood that wherever copper is referred to herein, the other heavy metals mentioned are to be considered as 25 included, slight modifications in technique necessitated by different melting points, etc. being, of course, necessary.

Even the presence of copper in relatively massive but always non-molten form makes for 30 readier alloying, but I prefer that the copper or other metal is added in more finely divided form 35 and well dispersed in one or both of the reacting constituents. The term "dispersed" is not herein used in the technical sense as employed in colloid chemistry, but in the more general sense of subdivision ranging from granular or filamentous condition to the molecular subdivision of solution and thorough admixture with the other reactants. I prefer powdered metal; and this can be made quite economically by aqueous electrolysis, or by reduction of the metallic oxides by 40 hydrogen, carbon monoxide, carbon, etc. For example, ground mill scale provides an excellent, inexpensive raw material for reduction to fine copper powder of the desired type.

My experiments indicate that the reduction of 45 the beryllium compound in the presence of such dispersed copper, as indicated, takes place most readily when a halide, or a mixture of halides of beryllium is reduced by a metal more electropositive than beryllium. It is known that the rela- 50

5

15

20

25

30

35

40

45

50

55

tive electropositivity of beryllium and other metals involved in this process varies in accordance with the compounds in which such metals appear. It is, therefore, to be understood that 5 the term "electropositive" and terms of similar import refer to the characteristic as exhibited in the case of the compounds in question. For example, beryllium chloride can be reduced by means of metallic sodium, the reactions being 10 initiated at about 500° C., or even lower, in the presence of dispersed copper. I prefer to carry out this reaction in a fused medium, with agitation. By employing a fused medium I am able to secure good contact between the heavy metal 15 and the beryllium compound so that wherever reduction of the beryllium compound occurs, by reason of contact with the reducing metal, the nascent beryllium can immediately contact the heavy metal. The fused medium serves not only 20 as a diluent and means of transmitting heat and dispersing the beryllium compound, heavy metal and, in some cases, the reducing agent, but also as a dispersion medium for the alloy of beryllium and heavy metal whereby to prevent any possible 25 occlusion of unreacted materials by the alloy. Any alkali halide or alkaline earth halide or any mixture of one or more thereof is suitable as a reaction medium. These compounds are not miscible with the resulting alloys and 30 therefore permit ready separation by gravity of the molten alloy. Sodium chloride, calcium chloride and sodium fluoride are particularly well suited for the purpose, as will appear. Many of the alkali and alkaline earth halides are impractical 35 on account of their high cost, although theoretically suitable. Still other substances may be used as dispersion media. I have made no attempt to determine exhaustively the substances which can be used, but it may be stated generally 40 that any substance, which is molten at the desired temperatures and is inert to or does not react harmfully with the reacting substances or products of the reaction and lends itself to ready separation after the reaction, is suitable. It is 45 not necessary to use any dispersion medium in addition to the reactants since the beryllium compound itself may be fused and act as a dispersion medium for the other materials. It is, however, desirable to have the dispersion medium 50 since the beryllium compounds are apt to volatilize excessively if the temperature goes much above their melting points. In the case of a compound such as sodium beryllium fluoride, the sodium fluoride component may be regarded 55 as the dispersion medium.

In the case of the reduction of beryllium chloride in the presence of dispersed, solid copper by means of metallic sodium it is desirable to use fused sodium chloride as a dispersion medium. 60 The double salt sodium beryllium chloride ( $Na_2BeCl_4$ ) is formed which greatly reduces the volatility of the beryllium chloride. Thus while the boiling point of beryllium chloride is about 475° C., the double salt remains substantially un- 65 volatilized at 800° C.

As stated above, I reverse the trend of the art by going to lower instead of higher temperatures. I am able to effect the alloying of beryllium with the heavy metal at temperatures even below the 70 melting point of the alloy, as well as at temperatures between the melting points of the alloy and the heavy metal constituent thereof. As a practical matter it is advantageous to start the reaction at a temperature well below the melting 75 point of the alloy and allow the heat liberated

by the reaction to carry the temperature thereabove. After the reaction is complete it is desirable to elevate the temperature above the melting point of the heavy metal so as to incorporate any small particles of unreacted heavy metal and produce a homogeneous product. This step 5 may include the addition of a further quantity of the heavy metal or of some other metal, if desired. By intentional dissipation of the heat of reaction it is possible to complete the reaction 10 at a temperature below the melting point of the beryllium-heavy metal alloy. If such procedure is followed, the temperature should be raised, after the reaction is complete, to a point above the melting point of the alloy, in order to fuse and 15 coalesce the particles thereof.

Equally successful is the use of fluorides of beryllium, either the double fluorides such as  $Na_2BeF_4$  or the monofluoride,  $BeF_2$ . This may be carried out with copper or other heavy metal 20 in a dispersion medium consisting of sodium fluoride, sodium chloride, calcium chloride or other alkali or alkaline earth halide, or, as previously shown, without any additional dispersion medium. If sodium fluoride is employed with beryllium fluoride, the double salt is formed as in the case of the chlorides and with similar advantage. These compounds can be reduced with sodium, calcium, or even magnesium. In the last-mentioned case, a ternary alloy is formed; and this 25 has direct advantages of its own even over the binary beryllium-heavy metal alloy. However, if only the binary alloy is desired, the ternary may subsequently be held above the boiling point of magnesium for a time sufficient to volatilize 30 out that metal and retain only the binary alloy. 35

A further modification of my invention permits the union of the reducing metal with the alloying metal, the basic principle of dispersion being maintained. For example, a fluoride of the 40 above-mentioned type may be reduced by a copper-calcium alloy. Using an alloy of 40% calcium content will yield, after reaction, an alloy of approximately 12-15% beryllium, ideal as a master alloy for dilution with further copper to the 2-3% 45 beryllium content which is commercially most desirable.

The same principle is ready applicable, to create a silver-beryllium alloy, by reducing beryllium chloride (preferably in combination with 50 sodium chloride) by a sodium-silver alloy.

It is manifest that the readiness of alloying, in light of what I have shown above, will vary with the particle size of the alloying metal and that fair results may be had from the use of a 55 relatively coarse dispersion of the heavy metal; practical considerations, however, dictate that the heavy metal added for alloying be in a condition to measure no more than approximately 0.1 of an inch each in at least two of its dimensions, 60 and preferably in all three. As already stated, I prefer truly powdered metal; and ranges of 50 mesh to 200 mesh have proven eminently satisfactory for the purpose. However, a state of subdivision less fine may be successfully used, particularly where vigorous agitation is employed. 65

The process, unlike any hitherto in actual practice for beryllium or its alloys, can be made fully continuous. For example, beryllium fluoride, made best by decomposition of the double ammonium beryllium fluoride, either in situ or separately, is added continuously to a bath of sodium fluoride or related fluorides, and simultaneously, there is continuous addition of copper powder and of the reducing metal, sodium. The bath is 70 75

preferably held at a temperature above the melting point of the copper-beryllium alloy to be made, and below the melting point of copper. As excess sodium fluoride forms in the bath, it can be bled off and a continuous flow of copper-beryllium alloy can be tapped from the bottom of the reaction receptacle. The same process is possible using beryllium chloride and sodium chloride.

It should be noted that it is possible to hold the bath itself at a temperature above the melting point of the heavy metal, provided such metal is contacted with the nascent beryllium before the particles of heavy metal can melt and coalesce. I therefore wish it understood that where bath temperatures are herein specified as below the melting point of the heavy metal, such expressions are not to be strictly construed but are to be given sufficient scope to cover such possible variations, within the spirit of my invention.

20 The process holds particular advantages over the present standard procedures, for alloying beryllium with iron, nickel and even copper by reason of the possibility of working at temperatures lower than the melting points of these 25 metals, temperatures at a suitable working range above the melting points of these metals being undesirably high and difficult to control.

The percentage of beryllium in the alloy can readily be regulated by proportioning the beryllium compound and the reducing agent in relation to the other metal present. It is generally convenient to produce the alloy with higher percentages of beryllium than is intended to be used in the final product and then to dilute the alloy 35 thus obtained by melting it with a suitable additional quantity of the other metal.

#### Examples

(1) One hundred thirty parts by weight of sodium beryllium fluoride, such as results from the interaction of beryl with an alkali silicofluoride, are introduced into a bath of fused sodium fluoride, or fused sodium-chloride. One hundred seventy five parts of copper powder are added with agitation. Continuing the agitation, fifty parts by weight of metallic sodium are added piecemeal. The reaction is preferably carried out in equipment of chromium-iron because of the corrosive properties of the reacting compounds, although iron or steel equipment can be used. The temperature at the beginning of the reaction is just above the fusion point of the bath and is maintained at the desired low temperature by loss of heat to the surroundings, which can be determined either by the construction of the equipment or by the rate at which the sodium is added or partly by each. Preferably the temperature is kept below the melting point of the alloy produced but may be between that temperature (which varies according to the composition of the alloy) and the melting point of copper. After the reaction is complete, the temperature is raised to about 1100° C. whereby to form a homogeneous alloy of beryllium and copper which is about five percent beryllium and to volatilize any excess sodium present. The temperature may optionally be kept down by the addition during the latter part of the reaction of a further quantity of from one hundred to two hundred parts by weight of copper either in powder or granular or even relatively massive form whereby to give an end product of from two to three percent beryllium, the temperature being raised after the reaction is complete to about 1100° C. to give a homogeneous product.

(2) Eighty parts by weight beryllium chloride are brought to fusion temperature. One hundred seventy five parts of copper powder are added with agitation. Continuing the agitation, fifty parts by weight of metallic sodium are added 5 piecemeal and sufficiently slowly to avoid a rise in temperature to a point above the melting point of copper before the reaction is substantially complete.

(3) One hundred thirty parts by weight of sodium beryllium fluoride are introduced into a fused bath of sodium fluoride or sodium chloride and one hundred ten parts by weight of copper calcium alloy in powder form and containing forty percent calcium, are added, with agitation, 15 and piecemeal. In this case the other conditions and procedure are the same as in the first example. The copper-calcium alloy can be handled more readily than sodium and contains the necessary copper. This procedure therefore possesses 20 some advantages.

In both the above examples eighty parts of beryllium chloride can be substituted for the sodium beryllium fluoride. The examples given indicate desirable procedures, but, obviously, a 25 great many variations as to quantity, temperature etc. are possible and numerous selections of reacting materials and end products can be made, all within the spirit and scope of my invention. I therefore wish it understood that I 30 am limited only in accordance with the appended claims and the prior art.

Having thus described my invention, what I claim is:

1. Process of alloying beryllium with another 35 metal which alloys therewith comprising dispersing a reducible beryllium compound and such other metal in finely divided solid form in a fused dispersion medium at a temperature below the melting point of such other metal and 40 contacting the dispersed substances with a reducing agent for the beryllium compound whereby to cause contact of the nascent beryllium with the small particles of said other metal, the temperature, however, being sufficient to effect 45 said alloying.

2. Process of alloying beryllium with one or 50 more metals selected from the group consisting of copper, iron, nickel, cobalt and silver, comprising dispersing a beryllium halogen compound and said metal or metals in finely divided form, in a fused dispersion medium selected from the group consisting of the alkali and alkaline earth halides and mixtures thereof, at a 55 temperature below the melting point of said metal or metals but sufficient to effect the alloying, and adding a beryllium reducing agent.

3. Process of alloying beryllium with another 60 metal which alloys therewith comprising dispersing a reducible beryllium compound and such other metal, the latter being in finely divided solid form, in a fused dispersion medium immiscible with the resulting alloy, at a temperature below the melting point of such other metal and contacting the dispersed substances 65 with a reducing agent for the beryllium compound whereby to cause contact of the nascent beryllium with the small particles of said other metal, the temperature being sufficient to effect 70 the alloying.

4. The process of forming beryllium-copper 75 alloys comprising reacting a beryllium halogen compound with a metal more electropositive than beryllium in the presence of finely divided solid copper.

5. The process of forming beryllium-copper alloys comprising reacting a beryllium halogen compound with a metal more electropositive than beryllium in the presence of finely divided solid copper, said beryllium compound and said copper being dispersed in a fused dispersing agent of the group consisting of the alkali and alkaline earth halides.
6. Process of alloying beryllium with a metal alloyable therewith comprising dispersing said metal in solid form in a fused, reducible compound of beryllium and contacting the resulting mixture with a reducing metal at a temperature below the melting point of said alloyable metal but sufficient to effect the alloying.
7. The process of forming beryllium-copper alloys comprising reacting a beryllium halogen compound with a reducing metal in the presence of finely divided solid copper.
8. The process of forming beryllium-copper alloys comprising reacting sodium beryllium fluoride with magnesium in the presence of finely divided solid copper.
9. The process of forming beryllium-copper alloys comprising reacting beryllium chloride with metallic sodium in the presence of finely divided solid copper.
10. The process of forming beryllium-copper alloys comprising reacting a beryllium halogen compound with a metal more electropositive than beryllium in the presence of finely divided solid copper, the temperature of the reaction being maintained below the melting point of the copper.
11. The process of forming beryllium-copper alloys comprising reacting a beryllium halogen compound with a metal more electropositive than beryllium in the presence of finely divided solid copper, the temperature of the reaction being maintained below the melting point of the copper until the reaction is substantially complete when the temperature is raised to precipitate the alloy.
12. The process of forming beryllium-copper alloys comprising reacting a beryllium halogen compound with a metal more electropositive than beryllium in the presence of finely divided solid copper, the temperature of the reaction being maintained below the melting point of the copper and preferably close to the melting point of the alloy.
13. The process of forming beryllium-copper alloys comprising reacting a beryllium halogen compound with a metal more electropositive than beryllium in the presence of finely divided solid copper, starting the reaction well below the melting point of the alloy, and allowing the temperature to rise above the melting point of the alloy and then elevating the temperature above that of the copper.
14. The process of forming beryllium-copper alloys comprising reacting a beryllium halogen compound with a metal more electropositive than beryllium in the presence of finely divided solid copper, starting the reaction well below the melting point of the alloy, allowing the temperature to rise above the melting point of the alloy and then elevating the temperature above that of the copper, and adding additional solid copper in a suitable state of division.
15. The process of forming beryllium-copper alloys comprising reacting a beryllium halogen compound with a metal more electropositive than beryllium in the presence of finely divided solid copper, and adding additional solid copper in divided state after the reaction is complete.

MENAHEM MERLUB-SOBEL.